

## UNITED STATES PATENT OFFICE

2,422,993

MANUFACTURE OF THREADS, FILAMENTS,  
FILMS, AND THE LIKE FROM ALGINATESErnest Edward Tallis, Meriden, England, assignor  
to Courtaulds Limited, London, England, a  
British companyNo Drawing. Application December 8, 1943, Serial  
No. 513,465. In Great Britain February 19,  
1943

1 Claim. (Cl. 18—54)

1

This invention relates to the manufacture of threads, filaments, and the like, which I will hereinafter refer to as "threads," from alginates. It is known that when spinning a solution of sodium alginate into a spinning bath containing acid, the threads, which are gelatinous, tend to adhere to one another and it has been proposed in British Patent 541,848, which corresponds to U. S. Speakman 2,371,717, to coat the filaments with oil during or immediately after coagulation and before they have had the opportunity of adhering together, and it has also been proposed to emulsify the oil by means of an addition of a cationic emulsifying agent, such as cetyl pyridinium chloride.

I have now found that threads and the like can be obtained from sodium alginate by spinning a solution of this latter into a bath containing a salt of an alkaline earth, such as calcium chloride, a small quantity of a cation-active compound such as cetyl pyridinium chloride and a small proportion of an organic acid such as acetic acid, in the substantial absence of free mineral acid. By this process I am able to obtain alginate threads which do not adhere to one another without it being necessary to add oil to the spinning bath.

The proportion of organic acid present should not be so great that any substantial quantity of alginic acid is present in the free state; suitable proportions are, for instance from 0.1 per cent to 5 per cent of acetic acid. With regard to the cation-active compound employed I have found that from 0.01 per cent to 0.1 per cent in the spinning bath is a suitable range, but larger quantities may be used, provided no substantial proportion thereof is salted out by the calcium chloride.

The following examples illustrate the nature of the present invention, although the invention is not restricted to these examples.

## Example 1

A solution containing 6.4 per cent of sodium alginate is extruded through a jet containing 20 holes into a bath containing 5 per cent of calcium chloride, 0.2 per cent of acetic acid and 0.05 per cent of cetyl pyridinium chloride at 40° centigrade. The thread produced is passed over two godets in such a manner that it is stretched 37

2

per cent and collected in a spinning box. The yarn thus obtained is reeled into skeins and washed with a solution of 0.1 per cent of calcium chloride at 80° centigrade. The skeins are dried at room temperature and conditioned at 65° relative humidity. The dry yarn is free from stuck filaments.

## Example 2

The conditions of spinning are the same as in Example 1 except that the spinning bath contains 5 per cent of calcium chloride 0.2 per cent of acetic acid and 0.02 per cent of undecylglycoline hydrochloride and is used at 27° centigrade. The yarn is washed with a solution containing 0.1 per cent of calcium chloride at 85° centigrade, air-dried and conditioned. The dry yarn is free from stuck filaments.

If in either of the foregoing examples the liquid used for washing the threads contains traces of alkali metals and/or magnesium, a small proportion, say 0.02 per cent to 0.05 per cent of a cation-active substance should be added to the washing liquid.

## 25 What I claim is:

A process of producing alginate threads free from stuck filaments which comprises extruding a solution of sodium alginate through a multi-hole jet into a coagulating bath consisting of water, about 5% of calcium chloride, from 0.01% to 0.10% of cetyl pyridinium chloride and from 0.1% to 5% of acetic acid and thereafter collecting the threads formed in a centrifugal spinning box.

35 ERNEST EDWARD TALLIS.

## REFERENCES CITED

The following references are of record in the file of this patent:

## 40 UNITED STATES PATENTS

| Number       | Name              | Date          |
|--------------|-------------------|---------------|
| 2,125,031    | Polak et al. .... | July 26, 1938 |
| 2,145,855    | Bley ....         | Feb. 7, 1939  |
| 45 2,371,717 | Speakman ....     | Mar. 20, 1945 |

## FOREIGN PATENTS

| Number     | Country            | Date          |
|------------|--------------------|---------------|
| 50 767,875 | France ....        | May 7, 1934   |
| 541,848    | Great Britain .... | Dec. 15, 1941 |